

1

3,392,176

**SOLVENTLESS COATING VEHICLE AND  
PROCESS FOR PREPARING IT**

David Eric Tweet, Minneapolis, Minn., assignor to  
Cargill, Incorporated, a corporation of Delaware  
No Drawing. Filed Jan. 2, 1964, Ser. No. 335,425  
7 Claims. (Cl. 260—404.8)

**ABSTRACT OF THE DISCLOSURE**

A 100 percent solids vehicle comprising the reaction product of an adduct formed by reacting 2-hydroxymethyl-5-norbornene, trimethylolpropane diallyl ether, and either maleic acid, maleic anhydride, or fumaric acid at an elevated temperature, and a drying oil, the reaction product being formed by blending the adduct and the drying oil at an elevated temperature.

The present invention generally relates to a coating vehicle, and more particularly relates to a 100 percent solids vehicle for use in coatings such as paints, varnishes and the like.

Various vehicles are known for use in coating formulations such as paints and varnishes and, in the past, drying oils, e.g., linseed oil and soybean oil, have been employed alone as coating vehicles, in the absence of other constituents. The drying oils set or dry to form hardened films upon exposure to air and/or heat due to oxidation and/or polymerization of the oils. However, the use of drying oils alone as coating vehicles has certain limitations since the coating films formed upon drying of the oils do not have a high degree of hardness and best weather resistance. Accordingly, in order to provide coating vehicles having improved hardness and weather resistance, various other constituents are added to the drying oils along with thinners. The thinners are volatile materials, such as water or an organic compound, e.g., benzene, turpentine, or other light organic solvent which, when combined with the drying oils and other constituents, provide a mobile coating vehicle having the desired coating characteristics. The use of volatile thinners is generally necessary to impart mobility and fluidity to the coating vehicle and/or coating formulation containing additional agents and other constituents, since the addition of these materials, which are necessary to provide durable coatings, having the desired characteristics, generally cause the coating vehicle and/or coating formulation to be so viscous as to be unsuitable for application with a brush or spray gun. When the coating formulation containing the volatile thinner is applied to a surface and allowed to dry the thinner evaporates, exposing the drying oils and other constituents in the formulation to the atmosphere and causing drying of the coating to a hard, weather resistant surface.

There are certain disadvantages in the use of coating vehicles which include vaporizable thinners or other volatile constituents. In this connection, if the coating vehicle comprises a substantial amount of vaporizable material which evaporates during drying, this material does not contribute to the ultimate body or thickness of the dried coating. Thus, the use of volatile thinners generally necessitates the application of two or more coatings in order to provide complete covering of the surface to be coated. Moreover, the volatile constituents in the coating vehicle may evaporate either before or after preparation of the coating formulation so that the coating vehicle does not have the desired characteristics upon application. Problems arise in connection with shipping and/or storage of organic thinners or other volatile constituents.

2

In an attempt to overcome the disadvantages associated with the use of volatile thinners and other constituents in coating vehicles, 100 percent solids vehicles have been formulated. A 100 percent solids coating vehicle is considered to be a vehicle which is free from vaporizable constituents under ambient conditions. Such a vehicle should provide desired hardness in the coating when applied, and should also provide suitable weather resistance and durability. At the same time, the 100 percent solids vehicle must be sufficiently mobile under ambient conditions that it may be applied to the surface to be coated by brush or by spray gun.

Generally, the 100 percent solids coating vehicles presently known provide a sufficient degree of physical hardness and weather resistance to coatings only when the coating is oven dried or baked at an elevated temperature. The available 100 percent solids vehicles do not provide air dried coatings, i.e., coating dried by exposure to the atmosphere at ambient conditions, which have the desired physical hardness and weather resistance.

One example of a 100 percent solids vehicle suitable for use where the coating is oven baked is described by United States Patent No. 2,867,593. However, the 100 percent solids vehicle described in Patent No. 2,867,593 is not capable of providing a suitable air-dried coating having the desired physical properties.

It is the principal object of the present invention to provide an improved vehicle for coating formulations. It is a further object to provide a 100 percent solids coating vehicle which, upon drying, provides a coating having desired hardness and weather resistance under ambient conditions. An additional object is to provide a 100 percent solids coating vehicle for use in coating formulations which provides increased coating film thickness upon normal application.

Further objects and advantages of the present invention will become apparent from the following detailed description.

Generally, the coating vehicle of the present invention comprises a reaction product of (1) an adduct of (a) 2-hydroxymethyl-5-norbornene (hereinafter sometimes referred to as Cyclol), (b) trimethylol propane diallylether and (c) maleic acid or anhydride and/or fumaric acid; and (2) a drying oil. The adduct generally comprises equal molar amounts of its constituents. Other known non-volatile constituents designed to modify or augment the characteristics of the coating vehicle may be mixed with the reaction product. More specifically, the coating vehicle of the present invention is a 100 percent solids vehicle comprising a reaction mixture of Cyclol, trimethylol propane diallylether maleate and/or fumarate, and from about 40 percent to about 60 percent by weight thereof of a drying oil.

2-hydroxymethyl-5-norbornene, more commonly known by its trade name "Cyclol," is an unsaturated monohydric alcohol having the following physical properties:

TABLE I

|                                     |                                                                                       |
|-------------------------------------|---------------------------------------------------------------------------------------|
| Molecular weight                    | 124.                                                                                  |
| Color APHA                          | Maximum 20.                                                                           |
| Boiling point (760 mm. Hg)          | 205° C.                                                                               |
| Freezing point                      | -11.5° C.                                                                             |
| Flash point, open cup               | 84° C.                                                                                |
| Specific gravity (25° C.)           | 1.022.                                                                                |
| Refractive index, N <sup>25</sup> d | 1.4994.                                                                               |
| Viscosity                           | 55 cps.                                                                               |
| Solubility                          | Organic solvents;<br>insoluble in cold<br>water; slightly<br>soluble in hot<br>water. |

Cyclol may be reacted with equimolar amounts of either maleic acid or anhydride or fumaric acid, and a particular monohydric ether in order to provide an adduct which can be further reacted with drying oils to form a 100 percent solids coating vehicle which can be air dried under ambient conditions to form a coating film having desirable hardness and resistance characteristics.

It has been discovered that in order to provide a mobile 100 percent solids vehicle that can be dried under ambient conditions, it is necessary to employ a particular ether as a reactant in the formation of the adduct. One such ether is trimethylol propane diallyl ether (TMPDAE). TMPDAE is a monohydric alcohol having the following chemical structure:



TMPDAE is soluble in acetone, methanol, ethyl acetate, n-butanol and benzene, but is insoluble in water.

Cyclol trimethylol propane diallyl ether maleate or fumarate may be formed by reacting together equimolar amounts of Cyclol, TMPDAE and either maleic acid or anhydride or fumaric acid, or mixtures thereof, at an elevated temperature of between about 300° F. to 500° F., preferably about 400° F., to an acid value of 2 to 20, and preferably an acid value of 10. Any unreacted materials remaining are preferably removed from the adduct by steam stripping. It is contemplated that the adduct may be prepared according to other equivalent processes and the exact mode of preparation of the adduct is not considered to be an essential part of the present invention.

The 100 percent solids vehicle is formed by blending together and reacting a Cyclol adduct with a drying oil or a mixture of drying oils. It has been found that superior air dried coating films are obtained when the drying oil is present in an amount of 66 percent to about 150 percent by weight of the adduct, although it is contemplated to employ about 25 percent to about 400 percent of the drying oils in certain instances. Known drying oils may be employed to form the 100 percent solids vehicle of the present invention. Specific examples of drying oils include linseed oil, safflower oil, dehydrated castor oil, soybean oil and mixtures thereof.

The blend of the adduct and the drying oil is heated at a temperature between about 350° F. to about 500° F., preferably about 420° F., until a sample thereof is clear at room temperature. The precise reaction that occurs during the heating of the adduct and drying oil blend is not completely understood, and it is not clear whether polymerization occurs. However, it is known that if the blend is heated at an elevated temperature until a sample is clear at room temperature, a particularly desirable 100 percent solids vehicle is obtained. As with the preparation of the adduct, the precise manner of reacting the adduct and drying oil is not considered critical, so long as a method of manufacture is selected that is equivalent to that described above.

It is preferable to add a stabilizer to the 100 percent solids vehicle in order to stabilize the vehicle in the presence of the usual paint driers, e.g., cobalt naphthenate or manganese driers. One suitable stabilizer is azo-bisisobutyronitrile.

100 percent solids coating vehicles of the type described herein may be incorporated in suitable coating formu-

lations and dried under ambient conditions to provide coating films having good physical hardness characteristics and resistance to weathering and abrasion. It is apparent that the coating vehicle may also be employed in coating formulations that are baked, if this is desired.

Certain tests have been conducted on the coating vehicles of the invention after drying to hardened films in order to determine the physical characteristics of the films. The hardness of the films, after various periods of drying, were determined by the standard Sward hardness of a 1.5 mils thick film. The brittleness of the films was tested by a standard  $\frac{1}{8}$  inch mandrel test as described in Gardner and Sward, Physical and Chemical Examination of Paints, Varnishes, Lacquer, and Colors, 10th Edition, 1946, at page 171. In accordance with the mandrel test a one mil thick film of the coating vehicle is applied to a  $\frac{1}{32}$  inch thick tin plate and air dried under ambient conditions for 72 hours. In order to pass the mandrel test the film should not crack when the plate is bent 180° over a  $\frac{1}{8}$  inch mandrel.

The reverse impact test is the number of foot pounds necessary to crack or fracture a one mil thick film applied to a  $\frac{1}{16}$  inch cold rolled steel plate that has been dried for 72 hours when struck on the reverse side by a Gardner impact hammer.

The mar resistance of the coating film was determined by striking the film a sharp glancing blow with the fingernails. In order to pass the mar resistance test, the film should not exhibit marks of any kind when struck with the fingernails.

#### Example I

A 100 percent solids vehicle is formed by reacting one mol of Cyclol, one mol of trimethylol propane diallyl ether and one mol of maleic anhydride at 400° F. to an acid value of 10 to form a Cyclol adduct. Any unreacted materials are stripped from the Cyclol adduct by heating.

The Cyclol adduct is blended with 100 percent by weight of the adduct of linseed oil and the blend is heated at 420° F. until a sample thereof is clear at room temperature. The coating vehicle thus formed is cooled to room temperature and 0.33 percent of azo-bisisobutyronitrile is added to stabilize the coating vehicle in the presence of driers.

The coating vehicle is mobile, having a viscosity of 3.0 poises, measured by the standard Gardner-Holdt viscosity tubes, and when mixed with various pigments and other constituents of coating formulations, provides a coating composition that is easy to apply and which dries rapidly in air to form coating films of good physical properties.

#### Example II

A coating vehicle is prepared in accordance with Example I except that linseed oil in an amount of 150 percent by weight of the Cyclol adduct is employed. The coating vehicle is mobile, having a viscosity of 1.6 poises, measured by the standard Gardner-Holdt viscosity tubes. The coating vehicle of this example can be incorporated in various coating formulations to form air dried films of acceptable physical characteristics.

The coating vehicles of Examples I and II are mixed with 1 gram per 100 grams of vehicle of cobalt naphthenate drier and are employed to form air dried films on various surfaces and are subjected to the previously described tests to determine the physical characteristics of the dried films. The results are set forth in the following table:

TABLE II

| Example No.: | Drying Time, Hours |           |            | Sward Hardness of 1.5 mils film |       |       | Reverse Impact Test, inch/lbs. | Mandrel Test | Mar Resistance |           |           |
|--------------|--------------------|-----------|------------|---------------------------------|-------|-------|--------------------------------|--------------|----------------|-----------|-----------|
|              | Set To Touch       | Tack Free | Print Free | 24 hr.                          | 1 wk. | 2 wk. |                                |              | 24 hr.         | 48 hr.    | 1 wk.     |
| 1-----       | 3.2                | 4.2       | 5.0        | 4                               | 18    | 30    | 36                             | Fail.....    | Pass.....      | Pass..... | Pass..... |
| 2-----       | 6.6                | 8         | 9.2        | 2                               | 12    | 18    | 160                            | Pass.....    | do.....        | do.....   | Do.....   |

Dried films of the coating vehicles are free from surface irregularity at all film thicknesses up to a wet film thickness greater than 3 mils. The films dry very rapidly under ambient conditions and exhibit good cohesion characteristics on all surfaces to which the vehicle is applied and can be used for coating metals as well as woods, plastics and other materials. The physical characteristics of dried films of the coating vehicles of Examples I and II set forth in Table II illustrate that a coating vehicle has been provided which, when air dried in the form of a coating film, has superior physical characteristics of hardness and resistance to cracking and abrasion.

It can be seen that a 100 percent solids vehicle has been provided which can be utilized to form dried films under ambient conditions of improved hardness and resistance. The coating vehicle may be employed in place of conventional volatile vehicles in most conventional coating formulations that are air dried. As used herein, the term "air dried" means that the coating film is dried under conditions approximating atmospheric temperature and pressure in the absence of elevated temperatures and forced oxidation.

Various of the features of the present invention are set forth in the following claims.

What is claimed is:

1. A 100 percent solids vehicle comprising a reaction product of (a) an adduct formed by reacting equimolar amounts of 2-hydroxymethyl-5-norbornene, trimethylolpropane diallylether, and a member selected from maleic acid, maleic anhydride or fumaric acid at a temperature of between about 300° F. and about 500° F. to an acid number of between about 2 and about 20, (b) between about 66 percent and about 150 percent by weight of the adduct of a fatty acid drying oil, the reaction product being formed by blending together and heating the adduct and the fatty acid drying oil at a temperature of between about 350° F. and about 500° F. until clear at room temperature.

2. A 100 percent solids vehicle comprising a reaction product of (a) an adduct formed by reacting equimolar amounts of 2-hydroxymethyl-5-norbornene, trimethylolpropane diallylether, and a member selected from maleic acid, maleic anhydride or fumaric acid at a temperature of between about 300° F. and about 500° F. to an acid number of between about 2 and about 20, and (b) between about 66 percent and about 150 percent by weight of the adduct of a fatty acid drying oil, selected from linseed oil, safflower oil, soybean oil and dehydrated castor oil, the reaction product being formed by blending together and heating the adduct and the fatty acid drying oil at a temperature of between about 350° F. and about 500° F. until clear at room temperature.

3. A 100 percent solids vehicle comprising a reaction product of (a) an adduct formed by reacting equimolar amounts of 2-hydroxymethyl-5-norbornene, trimethylolpropane diallylether, and a member selected from maleic acid, maleic anhydride or fumaric acid at a temperature of between about 300° F. and about 500° F. to an acid number of between about 2 and about 20, and (b) between about 100 percent and about 150 percent by weight

of the adduct of a fatty acid drying oil, selected from linseed oil, safflower oil, soybean oil and dehydrated castor oil, the reaction product being formed by blending together and heating the adduct and the fatty acid drying oil at a temperature of between about 350° F. and about 500° F. until clear at room temperature.

4. A 100 percent solids vehicle comprising a reaction product of (a) an adduct formed by reacting equimolar amounts of 2-hydroxymethyl-5-norbornene, trimethylolpropane diallylether, and a member selected from maleic acid, maleic anhydride or fumaric acid at a temperature of between about 300 F. and about 500 F. to an acid number of between about 2 and about 20, and (b) between about

10 66 percent and about 150 percent by weight of the adduct of linseed oil, the reaction product being formed by blending together and heating the adduct and the linseed oil at a temperature of between about 350° F. and about 500° F. until clear at room temperature.

5. A method for manufacturing an improved 100 percent solids vehicle, which method comprises, forming an adduct by reacting equimolar amounts of 2-hydroxymethyl-5-norbornene, trimethylolpropane diallylether and a member selected from the group consisting of maleic acid and anhydride and fumaric acid, at an elevated tem-

20 perature to an acid number of from about 2 to about 20, blending said adduct with about 66 percent to about 150 percent by weight of said adduct of a drying oil and heating said blend until clear at room temperature.

6. A method for manufacturing an improved 100 percent solids vehicle, which method comprises, forming an adduct by reacting equimolar amounts of 2-hydroxymethyl-5-norbornene, trimethylolpropane diallylether and a member selected from the group consisting of maleic acid and anhydride and fumaric acid, at a temperature of from about 300° F. to about 500° F. to an acid number of from about 2 to about 20, blending said adduct with about 66 percent to about 150 percent by weight of said adduct of a drying oil and heating said blend at a temperature of about 350° F. to about 500° F. until clear at room temperature.

7. A method for manufacturing an improved 100 percent solids vehicle, which method comprises, forming an adduct by reacting equimolar amounts of 2-hydroxymethyl-5-norbornene, trimethylolpropane diallylether and a member selected from the group consisting of maleic acid and anhydride and fumaric acid at a temperature of about 400° F., to an acid number of about 10, blending said adduct with about 66 percent to about 150 percent by weight of said adduct of a drying oil selected from the group consisting of linseed oil, safflower oil and dehydrated castor oil and heating said blend at about 420° F. until clear at room temperature.

#### References Cited

#### UNITED STATES PATENTS

3,192,061 6/1965 Wilson et al. 106—250

NICHOLAS S. RIZZO, Primary Examiner.

R. GALLAGHER, Assistant Examiner.